

# UNITED STATES PATENT OFFICE.

CHRISTOPHER C. TRINKLE, OF ROMNEY, INDIANA.

## COMPOUND FOR TEMPERING STEEL.

1,243,899.

Specification of Letters Patent. Patented Oct. 23, 1917.

No Drawing.

Application filed February 19, 1917. Serial No. 149,418.

*To all whom it may concern:*

Be it known that I, CHRISTOPHER C. TRINKLE, a citizen of the United States, residing at Romney, in the county of Tippecanoe and State of Indiana, have invented certain new and useful Improvements in Compounds for Tempering Steel, of which the following is a specification.

My invention relates to a compound for 10 tempering steel which is neither poisonous nor explosive and has for its object the production of a compound of the above described character and of a process of using the same and to this end my invention consists in a composition of matter composed of 15 the following constituents, combined in a pulverized state in the following proportions, namely:

|    |                     |          |
|----|---------------------|----------|
| 20 | Bicarbonate of soda | 2 quarts |
|    | Willow charcoal     | 2 quarts |
|    | Sal ammoniac        | 1 quart  |
|    | Sulfur              | 1 quart  |
|    | Copperas            | 1 quart  |
| 25 | Table salt          | 1 quart  |

These constituents are first to be pulverized, then combined in the proportions stated and then thoroughly mingled in their pulverized state by agitation.

In the use of my compound to temper any

article of steel I employ the following process, namely:

In each instance that part of the article of steel to be tempered is heated in the fire 35 to a cherry-red, then removed and covered with the compound by sprinkling or otherwise, then returned to the fire and slowly reheated to a cherry-red, then removed and bathed in warm water, then the temper is 40 drawn until a file takes hold regardless of color and then deposited in warm water until cool.

By the use of my compound in the manner stated articles of steel may be thoroughly 45 tempered and materially toughened by a common iron-worker.

In the above described compound and process of using the same I produce a new and useful invention for tempering steel, tool- 50 steel and steel-tools of every description.

What I claim as my invention and desire to secure by Letters Patent, is:

The herein described compound, comprising bicarbonate of soda, willow charcoal, 55 sal ammoniac, sulfur, copperas, and table salt, substantially as described and for the purpose specified.

CHRISTOPHER C. TRINKLE.

Witnesses:

ALBERT CALDWELL,

JOE R. CANINE.